

## UNITED STATES PATENT OFFICE.

FREDERICK M. BECKET, OF NEW YORK, N. Y., ASSIGNOR TO ELECTRO METALLURGICAL COMPANY, OF NEW YORK, N. Y., A CORPORATION OF WEST VIRGINIA.

## ZIRCONIUM STEEL AND PROCESS OF MAKING SAME.

No Drawing.

Application filed August 11, 1922. Serial No. 581,285.

To all whom it may concern:

Be it known that I, FREDERICK M. BECKET, a citizen of the United States, residing at New York, in the county of New York and State of New York, have invented certain new and useful Improvements in Zirconium Steel and Processes of Making Same, of which the following is a specification.

This invention relates to the art of steel manufacture, and comprises a process of treating high-sulphur steels whereby they may be rendered acceptable under the usual engineering specifications. The invention comprises also, as a novel product, a steel of high-sulphur content, said steel being nevertheless free from the so-called "red-shortness" which has heretofore been considered as a necessary characteristic of all such high-sulphur steels. These results are attained, in accordance with the present invention, by the addition of zirconium to the molten steel, optimum treating conditions being herein-after set forth.

As is well known, the deleterious effects of a high-sulphur content in steel are most apparent during rolling or forging at the customary high temperatures required by these operations. The term "red-shortness" applies to the tearing or cracking of the steel during such hot-working operations. The occurrence of "red-shortness" in a steel may, in aggravated cases cause the metal to break up completely under the rolls or hammer, just as though it were possessed of great brittleness; while in less severe cases the rolled or forged steel shows, upon inspection of its surface, cracks, fissures, or reticulated systems of seams, which in themselves are sufficient to cause the rejection of the material. High-sulphur steels exhibiting the less severe type of "red-shortness" may in numerous instances fail to show upon comparison with low-sulphur steels, any appreciable decrease in the values of those commonly determined mechanical properties,—such as tensile strength, percentage elongation, Izod number, etc., which are referred to measurements made in the cold; and especially is this true if the test-pieces from the high-sulphur steel are taken at

some distance from the surface of the rolled or forged metal so as to escape the major surface cracks or seams.

In consequence of the above-mentioned facts, it follows that the most reliable test of the efficacy of any given addition agent in counteracting the harmful effect of sulphur consists in an examination into the actual behavior of the steel under rolling or forging operations, and it has been by means of such experimental work that the beneficial effect of zirconium upon high-sulphur steel which forms the basis of the present invention has been most conclusively demonstrated.

In those cases among existing A. S. T. M. specifications for steel where a maximum sulphur content is given, the allowable limit ranges from 0.03% for chrome and chrome-vanadium automobile steel to 0.08% for commercial bar (carbon) steels of Bessemer grade. The limits which most frequently occur are from 0.04% to 0.05%, however. In the case of a number of A. S. T. M. specifications,—such as for instance carbon steel rails, splice bars, track bolts and spikes, structural steel for buildings, and concrete reinforcement bars, it is true that no limits for sulphur are specified. But in practice there are always allowable limits of sulphur assigned for any given steel, which limits are either the result of an agreement between manufacturer and purchaser or are voluntarily set by the manufacturer in accordance with his own previous experience with that particular grade of steel.

It is therefore not practicable for the purposes of the present invention arbitrarily to define what is meant by the term "high-sulphur steel". Not only does the maximum sulphur limit vary with the grade of steel produced and especially with the manganese content of the same, but this maximum practical limit depends largely upon the exact manner in which the metal is rolled or forged.

I regard as being within the scope of my invention the treatment of any steel with zirconium which results in an unmistakable improvement in those hot-working proper-

65

60

65

70

75

80

85

90

95

100

ties which are dependent upon the sulphur content, as well as the product thereby produced. In many cases, such application of zirconium makes possible the satisfactory 5 rolling or forging of steel which could not otherwise be worked owing to its high-sulphur content.

The use of zirconium as a deoxidizer, 10 solidifier, and scavenger of steel, as has often been proposed, as well as its use to counteract the embrittling effect of phosphorus ("cold-shortness") in high-phosphorus steels, as set forth in a co-pending application 15 of F. M. Becket, Serial No. 528,283, filed January 10, 1922, are to be clearly distinguished from that described herein, which contemplates the employment of this metal 20 for the specific purpose of improving its hot-working properties.

In the course of this investigation it has 25 been found that the beneficial effect of zirconium upon the hot-working properties of high-sulphur steels is in some way correlated with the fact, which we have observed, that in many if not indeed in all cases zirconium enters into chemical combination 30 with sulphur in the steel melt. While this zirconium-sulphur compound has not yet been isolated or definitely identified microscopically, its existence is demonstrated by 35 the effect of zirconium upon the amount of hydrogen sulphide evolved when the steel is treated with 1:1 hydrochloric acid in accordance with the usual evolution-titration method of analysis. From the results of 40 numerous analyses made on steels of different sulphur contents and treated with different amounts of zirconium, it has been established (a) that an acid-insoluble zirconium sulphide or zirconium-sulphur combination is formed; and (b) that only the 45 zirconium in excess of a definite quantity which appears to be of the order of 0.10—0.15% added zirconium takes part in this sulfid-forming reaction. In other words under the conditions employed in this investigation approximately 0.10—0.15% added zirconium was used up in the course of 50 other chemical reactions, probably involving the oxygen and nitrogen present in the melt.

The percentage of zirconium which must be added to the molten steel to obtain the maximum beneficial effects is determined by 55 a multiplicity of factors, including temperature and degree of oxidation of the steel bath; the composition of the steel; the composition of the alloy or aggregate containing zirconium which is used; the manner in 60 which the addition is made; and the type and severity of hot-working to which the steel is subjected before it is put into use in finished form. For example, in the manufacture of carbon steels containing around

0.12% sulphur, I now prefer to obtain the 65 desired beneficial results by the addition of from 0.15 to 0.50% zirconium calculated on the weight of the steel.

Our experiments have shown that the 70 above-described beneficial effect of zirconium is primarily due, not to the actual elimination of sulphur from the steel bath, but to the "fixation" of the sulphur by means of chemical combination with zirconium. As has 75 been stated, a zirconium-sulphur compound which is insoluble in 1:1 hydrochloric acid may be produced, so that an ordinary analysis of the treated steel for sulphur by means of the evolution-titration method might lead one to conclude that sulphur was actually 80 eliminated in amount indicated by the equation cited above. Gravimetric analysis, however, involving solution in and oxidation by nitric acid, followed by precipitation as barium sulphate, discloses the fact 85 that this apparent quantitative elimination of sulphur is due to the formation of a compound insoluble in 1:1 hydrochloric acid. Further investigation on this point 90 has revealed the fact that in addition to this quantitative elimination of sulphur, which is only apparent, there may be and very often is an actual elimination of sulphur 95 from the bath which in its extent depends upon a multiplicity of factors, chief among 100 which is the length of time the steel is held in the furnace or ladle subsequent to the addition of zirconium. This time element is associated with those progressive processes which result in the separation of lighter, non-metallic particles and globules from a fluid metal bath,—processes which are well-understood by those familiar with the art.

Whereas, therefore, actual "slagging off" 105 and elimination of the zirconium-sulphur compound depends upon the formation of said compound, this subsequent process of elimination of sulphur must not be regarded as an essential feature of the present invention, although it is a feature which is 110 advantageous and should be encouraged in practice.

The investigation into the treatment of 115 high-sulphur steels with zirconium has included the making of a number of heats of steel; the casting of ingots; the rolling and forging of ingots; and the machining and testing of various test-pieces. Equal weights 120 of molten steel were tapped from the furnace into two separate ladles in the case of each heat. The "A" ladle was in each case treated with silicon-zirconium and the "B" ladle with 50% ferrosilicon, each of the two additions being adjusted to correspond to the same amount of added silicon. The ladles of steel after treatment were teemed into tapered molds of the usual type and the two 125

ingots from each heat were rolled (or forged) under the same conditions of temperature and working.

As a typical example, the analysis of a 5 silicon-zirconium used in the course of the work is given as follows:

*Silicon-zirconium.*

|    |           | Per cent. |
|----|-----------|-----------|
| 10 | Zirconium | 44.53     |
|    | Silicon   | 50.77     |
|    | Iron      | 2.54      |
|    | Titanium  | 0.70      |
|    | Carbon    | 0.48      |

15 Since the effect of zirconium which is herein described consists in an improvement of "hot-working" properties and elimination of "red-shortness," it is not feasible to present the results of the investigation in 20 the form of tables or curves. For purposes of illustration, however, an account of the results obtained in the case of a typical heat will be given.

This heat of steel was poured into two 25 ladles, one ladle ("A") being treated with 0.15% zirconium and 0.18% silicon as silicon-zirconium and the other ladle ("B") with 0.18% silicon only, as 50% ferrosilicon. The steel had the following analysis:

|    | C    | Si   | Mn   | P     | S     |
|----|------|------|------|-------|-------|
| 30 | 0.44 | 0.15 | 0.28 | 0.018 | 0.075 |

The ingots were of slab form, with a 35 width equal to twice their thickness, and were rolled directly down to  $\frac{1}{2}$ " plate, without cross-rolling, in a commercial mill. The temperature of the heating furnace was maintained at 2010° F. The ingots were rolled to  $\frac{1}{2}$ " plate in about 6 passes, at a reduction from 33 $\frac{1}{2}$  to 100% greater than that 40 normally used, in order to emphasize any "red-shortness" present.

Inspection of the finished steel plate 45 showed the "A" or silicon-zirconium treated steel to be entirely free from cracks, seams, or other imperfections. The "B" plate, treated with the same amount of silicon but without zirconium, was badly broken up and splintered along the edges over the upper half (corresponding to the top of the original ingot) and contained several bad fissures along the edge of the lower half.

The above is one typical experiment selected from a number of similar experiments, in all of which the beneficial effect 55 of zirconium was unmistakable.

The above-described process will, it is believed, greatly increase the quantity of coking coal available for the production of blast-furnace coke, and also make available 60 for steel production a large tonnage of pig-

iron and scrap which is now considered "off-grade" because its sulphur content is above the limit set by specifications. The sulphur problem is one of the most serious 65 which the industry faces today, because of the fact that the open-hearth furnace process, which uses large percentages of scrap steel in its charge, is fighting a losing fight against the natural tendency toward the accumulation of scrap higher and higher in its sulphur content. This is due to several different factors, as follows: (1) the use of lower-grade coke both in blast-furnaces and in foundries; (2) the difficulty of eliminating sufficient sulphur in the open-hearth furnace and particularly in the acid open-hearth furnace to make up for the sulphur contained in the fuel which heats the furnace, and (3) the concentration of sulphur 70 in the steel bath due to oxidation of the steel during the melting-down stage.

Since the use of zirconium will do much toward alleviating this situation, the practical benefits of the present invention will 75 be obvious to those familiar with the art.

I claim:

1. Process of treating steels containing sufficient sulphur to cause red-shortness, comprising adding zirconium thereto in proportion sufficient to counteract to a substantial degree the detrimental effect of the sulphur. 80

2. Process of treating steels containing sufficient sulphur to cause red-shortness, comprising adding zirconium thereto in the proportion of about 0.15 to 0.50% zirconium, calculated on the weight of the steel. 85

3. Process of treating steels containing not less than 0.05% sulphur which comprises adding zirconium thereto in proportion sufficient to counteract to a substantial degree the detrimental effect of the sulphur. 100

4. As a new composition of matter, a high sulphur-steel containing zirconium. 105

5. As a new composition of matter, steel containing zirconium and upward of 0.05% sulphur. 110

6. As a new composition of matter, steel containing sulphur and zirconium, and characterized by relative freedom from red-shortness as compared with a steel of like composition free from zirconium. 115

7. As a new composition of matter, steel containing zirconium and upward of 0.05% sulphur, said steel characterized by relative freedom from red-shortness as compared with a steel of like composition free from zirconium. 120

In testimony whereof, I affix my signature.

FREDERICK M. BECKET.